

Patented Jan. 27, 1931

1,790,552

## UNITED STATES PATENT OFFICE

AUGUSTUS F. MEEHAN, OF CHATTANOOGA, TENNESSEE, ASSIGNOR TO MEEHANITE METAL CORPORATION, OF CHATTANOOGA, TENNESSEE, A CORPORATION OF TENNESSEE

### ALLOY FOR MANUFACTURE OF CAST IRON

No Drawing.

Application filed August 29, 1928. Serial No. 302,889.

The present invention relates to the treatment of metals, and, more particularly, to the treatment of molten metal in the manufacture of castings.

- 5    An object of the invention is to provide a process for the manufacture of castings of special strength and uniformity, such as will insure the quality sought in the finished castings.
- 10   Heretofore, when deemed essential, it has been the practice in the manufacture of grey iron castings to add to the molten metal a suitable agent in order to obtain the carbon in the desired forms.
- 15   In the breaking down of the iron carbide in the metal during solidification, ferro-silicon generally has been used as a graphitizing agent in order to provide the proper ratio of combined and graphitic carbon in the casting, and in a treatment of molten metal such as would upon solidification produce a casting white in fracture, into metal for castings the fracture of which would be grey, the use of the silicide substantially free from iron 20 is suggested in my Patent 1,499,068, granted June 24th, 1924.
- 25   My investigations have disclosed that the character of grey castings may be materially improved by the treatment of molten metal for making castings which would be gray but which ordinarily would have rather limited mechanical properties, through the introduction in the molten metal of a silicide substantially free from iron. It has been 30 found that a silicide of an alkaline earth metal, such as calcium or magnesium, or other alkaline earth metal, will materially improve the casting, even though it contains an amount of graphitic carbon that was not precipitated by the silicide referred to, and 35 would have been grey in fracture without the introduction of the silicide.
- 40   The introduction of such a silicide, even in molten metal which, when cast, ordinarily would be grey in character, is readily soluble and workable, and acts to precipitate additional carbon in spite of which the tensile and transverse strength will be materially increased. It has been found that the silicide 45 produces this effect in molten iron adapted to
- produce a casting containing approximately 3% of combined carbon, and even in iron containing less than 1% of combined carbon.
- 50   By the statement that the silicide is substantially free from iron, is meant that the iron content of the treating agent or alloy is relatively inconsiderable.
- 55   I have also found that in the production of castings, the silicide agent may be accompanied to advantage by a second alkaline earth metal, such as magnesium, strontium, barium, etc. For example, an alloy agent of calcium, silicon and an inconsiderable amount of iron may also include to advantage either magnesium or strontium or barium, etc.
- 60   The agents described above, when used separately or combined as alloys, have been found to be of increased or intensified value if accompanied by nickel, or aluminum, or chromium, or titanium or vanadium. In some instances, more than one of these elements may be employed to advantage; for example both nickel and chromium. The addition of this 65 second element, especially chromium has been found to increase the capacity of the metal to resist high pressures and temperatures. Also it increases the resistance to acids and acidic oil vapors.
- 70   The following alloys are given as examples of ones that have been found to be satisfactory:
- 75   *Example 1*
- |         | Per cent | 85    |
|---------|----------|-------|
| Calcium | 33       | to 35 |
| Silicon | 62       | to 65 |
| Iron    | 3        |       |
- 80   *Example 2*
- |          | Per cent | 90 |
|----------|----------|----|
| Calcium  | 33       |    |
| Aluminum | 8        |    |
| Iron     | 3        |    |
| Silicon  | 56       |    |
- 85   *Example 3*
- |         | Per cent | 95    |
|---------|----------|-------|
| Silicon | 53       | to 60 |
| Calcium | 32.60    | 35    |
| Nickel  | 3.60     |       |
| Iron    | 2.60     | 100   |

### Example 4

Calcium \_\_\_\_\_  
Magnesium \_\_\_\_\_  
Silicon \_\_\_\_\_

### Example 5

Silicon -  
Nickel -  
Magnesium -  
10 Calcium -

### Example 6

|    |          | Per cent    |
|----|----------|-------------|
|    | Silicon  | 53 to 60    |
|    | Calcium  | 32.60 to 35 |
| 15 | Nickel   | 2.60        |
|    | Chromium | 1           |
|    | Iron     | 3           |

These agents may be introduced into the molten metal, in any suitable manner, either in combination, i. e., as alloys, or separately. ordinarily the alloy or separate elements are reduced to relatively small particles, although the alloy may be used in brick or briquette form, and a few ounces of the same used to a small percentage of the metal treated. The agents may be added in the spout as the molten metal runs from the furnace, or thrown into the stream of metal where it enters the ladle from the spout, or else added to the metal in the furnace.

Although the percentages given in the foregoing examples may be varied considerably, it is to be understood that where reference is made in the specification and claims to the use of a silicide, such as calcium or magnesium silicide, I mean an amount of the same sufficient to produce an appreciable graphitizing effect. Since the molten iron will vary in its characteristics, the amount of silicide needed, in particular instances, will be governed accordingly, the silicide being used, of course, in sufficient amounts to produce the desired graphitizing effect.

45 to produce the desired graphitizing effect.  
By "molten white iron", I mean such molten iron as will produce castings substantially free from graphitic carbon. By "white iron" I mean such castings as are substantially free from graphitic carbon. By "gray  
50 molten iron" I mean such molten iron as will produce castings in which more or less graphitic carbon will be present. By "gray iron" I mean castings in which more or less graphite is present.

55 This application is a continuation-in-part of my application, Serial No. 199,419, cast iron and the method of making same, filed June 16, 1927, and which on September 4, 1928, matured into Patent 1,683,086.

60 I claim:

1. An alloy for use in the treatment of molten iron for making cast iron, comprising silicon in not less than approximately 50%, an alkaline earth metal in excess of 25%, a metal such as nickel from a substantial

65 metal such as nickel from a substantial

amount up to 5%, and a second alkaline metal of the calcium-magnesium group in a percentage somewhat less than one-half the percentage of the first alkaline metal.

2. An alloy for the use in the treatment of molten iron for making cast iron containing the following in substantially the proportions specified: silicon, 53% to 60%; calcium, 32.60% to 35%; nickel, 3.60%; iron, 2.60%. 75

3. An alloy for the use in the treatment of molten iron for making cast iron containing the following in substantially the proportions specified: calcium, 35%; magnesium, 9%; silicon, 56%.

4. An alloy for the use in the treatment of molten iron for making cast iron containing the following in substantially the proportions specified: silicon, 51%; nickel, 5%; magnesium, 9%; calcium, 35%. 85

In testimony whereof I have hereunto set my hand.

AUGUSTUS F. MEEHAN.

90

85

100

105

10

202

120

125

180